

## UNITED STATES PATENT OFFICE

BYRAMJI D. SAKLATWALLA, OF CRAFTON, PENNSYLVANIA

## FERROUS ALLOY

No Drawing.

Application filed October 29, 1927. Serial No. 229,792.

This invention relates to ferrous alloys and particularly to a ferrous alloy containing copper, silicon and aluminum. The copper and silicon impart to ferrous metal corrosion resisting properties in a high degree and together with chromium these elements have been utilized to produce some of the corrosion resisting steels such as described in the applicant's Patent No. 1,676,929 of July 10, 1928. For certain purposes, however, especially for resistance to scaling at high temperatures, expensive chromium can be eliminated and replaced by comparatively small percentages of aluminum.

According to the present invention, by the addition of about 0.1% to 2.00% aluminum to alloy steels or irons containing copper and silicon it has been found that steels or irons showing remarkable resistance to scaling and corrosion at high temperatures can be produced. By varying the copper content in such steels from 0.5% to 5.00% and the silicon content from 0.5% to 6.00% a series of alloys can be produced with varying degrees of non-corrosive properties at high temperatures. Such alloys can be produced with very low carbon contents but for the physical requirements of strength the usual carbon percentages occurring in steel, namely from 0.1% to about 2.00% can be utilized. Such steels can be fabricated by the usual steel making processes, obtaining material of sound physical characteristics and great degree of ductility. Such material can be forged into bars, rolled into sheets, etc. Such alloys can further be improved as to their physical characteristics by the proper heat treatment. Such materials can be obtained in the annealed condition or can be improved by the processes of quenching and drawing back, thus furnishing a very wide latitude of materials with different physical properties.

Besides the rolled and forged materials, cast materials of this composition resisting the action of high temperature can be obtained by allowing the carbon content to increase up to about 3.5%. Such cast materials can also be subjected to annealing or other heat treating processes whereby their

physical characteristics can be markedly improved.

Materials of this composition with the suitable carbon range are, therefore, very well adapted to the manufacture of internal combustion engine valves, carburizing boxes, electrical resistance heating elements, tools and rolls operating at high temperature and for other purposes where a metal is desired to resist scaling at a high degree of heat. Such materials are especially remarkable for retaining their physical strength at elevated temperatures.

For different purposes the percentages of copper, silicon and aluminum can be varied to suit the requirements as to scaling and to loss in physical strength at high temperatures. For extreme heat resisting purposes the amounts of silicon are increased up to the upper limit of 6.00%. The upper limit of aluminum up to 2% is also useful in bringing about non-scaling properties at high temperatures. In cases where chemically corrosive action from combustion gases, etc. is important a high copper content up to the upper limit of 5.00% is advantageous.

The various steels and irons according to this invention showing the properties above described can be produced by variation of the contents of silicon, copper and aluminum with the following limits:

Copper from 0.5% to 5.00%.

Silicon from 0.5% to 6.00%.

Aluminum from 0.1% to 2.00%.

In the above described ranges the carbon content can be either that of the steel range, namely; from 0.1% to 2.00%, or in the cast iron ranges from 2.00% to 3.50%. Also in the above described alloys no reference is made to the presence of other elements, such as manganese, sulphur, phosphorus, etc., always present in steels and cast irons as their presence to the usual extent does not interfere with the properties of the above described ferrous alloys. Further, any refining agents or alloys such as titanium, vanadium, zirconium, etc., added to these compositions to the extent as is ordinarily done in alloy steels does not change the characteristic properties of these ferrous alloys.

55

60

65

70

75

80

85

90

95

100

The present invention is not limited to the exact proportions set forth, as its preferred embodiment, but may be otherwise embodied within the scope of the following claims.

I claim:

1. A ferrous alloy containing from 0.5% to 5.0% copper, from 0.5% to 6.00% silicon, and from 0.1% to 2.00% aluminum, together with carbon within the range of cast iron, and characterized by its resistance to scaling and corrosion at high temperatures.
- 10 2. A cast iron alloy containing from 0.5% to 5.0% copper, from 0.5% to 6.00% silicon, and from 0.1% to 2.00% aluminum, together with carbon from 2.0% to 3.5%, and characterized by its resistance to scaling and corrosion at high temperatures.

In testimony whereof I have hereunto set my hand.

20 BYRAMJI D. SAKLATWALLA.

25

30

35

40

45

50

55

60

65